

## UNITED STATES PATENT OFFICE

2,556,373

## ALLOY STEELS FOR USE AT ELEVATED TEMPERATURES

Henry William Kirkby and Charles Sykes, Sheffield, England, assignors to Thos. Firth & John Brown Limited, Sheffield, England, a British company

No Drawing. Application April 14, 1950, Serial No. 156,044. In Great Britain August 23, 1949

2 Claims. (Cl. 75—125)

1

This invention relates to alloy steels for use at elevated temperatures.

To provide alloys having a high creep resistance at temperatures up to 800° C. the following range of composition has been proposed (see 5 British specification No. 577,892):

Carbon, up to 1.5%  
Nickel, 15.0 to 25%  
Chromium, 12.0 to 20.0%  
Molybdenum, 2.0 to 6.0%  
Copper, 2.0 to 6.0%  
Titanium, 0.25 to 2.0%  
Iron, remainder

The above alloy may also contain silicon up to 2%, manganese up to 2% and vanadium up to 1%.

The addition of cobalt to the above alloys, the cobalt and nickel proportions being respectively 7 to 40% and 25 to 15%—for the purpose of improving further the creep resistance properties—has also been proposed (see British specification No. 616,207), and in such alloys containing cobalt as proposed the substitution of columbium for the whole or part of the titanium content of the alloy has also been suggested.

A further prior proposal in connection with alloys resistant to creep relates to compositions embodying a lower range of nickel, together with cobalt 7 to 50% and columbium 0.5 to 2% interchangeable with titanium.

The elements cobalt and columbium are strategically rare and consequently their use in alloy steels presents an economic difficulty. The present invention seeks to provide an alloy having high creep resistance properties up to at least 700° C. without relying on either cobalt or columbium for these properties.

Alloys according to this invention lie within the following range of composition:

Carbon, up to 0.40%  
Silicon, up to 1.0%  
Manganese, up to 3.0%  
Chromium, 9 to 17.0%  
Nickel, 7 to 12.0%  
Molybdenum, 2 to 3.0%  
Tungsten, up to 3.0%  
Copper, 1.0 to 4.0%  
Titanium, 0.25 to 1.0%

Balance substantially iron with residual impurities in ordinary amounts.

The preferred range of composition is as follows:

Carbon, 0.15 to 0.30%  
Silicon, 0.20 to 0.40%

2

Manganese, 0.20 to 1.0%  
Chromium, 13.5 to 15.0%  
Nickel, 8.0 to 11.0%  
Molybdenum, 1.75 to 2.25%  
Copper, 2.0 to 2.75%  
Tungsten, 0-2.0%  
Titanium, 0.50 to 1.0%  
Iron, substantial remainder

10 In the present alloys importance is attached to the low nickel range of proportions and to the inclusion in the alloy of up to 3% of tungsten.

An alloy within the above preferred range of composition, after suitable heat treatment of 15 generally known character, gave the following results of stress to rupture tests:

| 20 | Stress (tons/sq. in.) at 700° C. | Hours to fracture |
|----|----------------------------------|-------------------|
|    | 17<br>19                         | 852<br>120        |

25 The above results compare favourably with known alloys containing considerable proportions of cobalt with or without columbium in addition. Moreover alloys according to the invention are superior to the previously proposed alloys (British specification No. 577,892)—already referred to—containing no cobalt or columbium, as is demonstrated by the following results of comparative stress-rupture tests:

| 35 | British Specification No. 577,892 | Temp., °C. | Stress, tons/sq. in. | Time (hours to fracture) |
|----|-----------------------------------|------------|----------------------|--------------------------|
|    |                                   | 650        | 18                   | 38                       |
| 40 | Present Application               | 700        | 12                   | 100                      |
|    |                                   | 700        | 19                   | 120                      |

45 The alloys according to this invention are particularly suitable for aircraft and gas turbine application.

We claim:

1. An alloy steel having high creep resistance properties as indicated herein at temperatures up to at least 700° C. and having a composition 50 characterised by the absence of cobalt and columbium and by the presence as essential constituents of carbon in effective proportion up to 0.4%, silicon in effective proportion up to 1%, manganese in effective proportion up to 3%, chromium 9 to 17%, nickel 7 to 12%, molyb-

denum 2 to 3%, tungsten in effective proportion up to 3%, copper 1 to 4%, titanium 0.25 to 1%, and balance substantially iron with residual impurities in ordinary amounts.

2. An alloy steel having high creep resistance properties as indicated herein at temperatures up to at least 700° C. and having a composition characterised by the absence of cobalt and columbium and by the presence as essential constituents of carbon 0.15 to 0.3%, silicon 0.2 to 0.4%, manganese 0.2 to 1%, chromium 13.5 to 15%, nickel 8 to 11%, molybdenum 1.75 to 2.25%, copper 2 to 2.75%, tungsten in effective proportion

up to 2%, titanium 0.5 to 1%, and iron the substantial remainder.

HENRY WILLIAM KIRKBY.  
CHARLES SYKES.

#### REFERENCES CITED

The following references are of record in the file of this patent:

#### UNITED STATES PATENTS

| Number    | Name     | Date          |
|-----------|----------|---------------|
| 2,402,814 | Hatfield | June 25, 1946 |
| 2,447,897 | Clarke   | Aug. 24, 1948 |